

Feb. 19, 1924.

N. K. DAVIS

**1,484,208**

## METHOD OF TREATING FIBER BEARING MATERIAL

Filed Nov. 30, 1921



*Inventor.*  
*Norris K. Davis.*

By *Acme & Teller*

*By* *Attorneys*

## UNITED STATES PATENT OFFICE.

NORRIS K. DAVIS, OF SAN FRANCISCO, CALIFORNIA.

## METHOD OF TREATING FIBER-BEARING MATERIAL.

Application filed November 30, 1921. Serial No. 518,912.

*To all whom it may concern:*

Be it known that I, NORRIS K. DAVIS, a citizen of the United States, residing at the city and county of San Francisco and State of California, have invented certain new and useful Improvements in Methods of Treating Fiber-Bearing Material, of which the following is a specification.

The hereinafter described invention comprises a method for the treatment of ores containing asbestosform serpentine, commonly known as asbestos, for the separation and recovery of the asbestos fiber from its enclosing rock. However, the invention is not restricted to the treatment of such material, inasmuch as it is adapted for the treatment of fiber bearing ores generally for the separation and recovery of the fiber therefrom.

In the treatment of asbestos bearing ores as carried out prior to the present invention, it has been customary to first crush the ore and to then pass the crushed material through screens and dusters for the separation of the fiber from the base or worthless material, after which the separated fiber is subjected to a cleaning action. This method of treatment not only requires the employment of expensive and heavy machinery, but the utilization thereof in the treatment of the fiber bearing ore for the recovery of the asbestos therefrom is such as to materially damage the fiber contained within the ore, and by reason of the injury thus done to the fiber in the breaking of the same destroys the length thereof and the value of the recovered fiber is materially lessened for use in the industrial arts.

By the use of the present invention, which dispenses with the employment of the hitherto employed crushing mechanism, the screening, dusters and cleaning means, I am enabled to make a recovery of the asbestos fiber from its enclosing rock without breaking down or destroying the length of the liberated fiber, thereby producing asbestos fiber of substantial uniformity and of considerable tensile strength and of a length capable of being spun into threads for the manufacture therefrom of asbestos cloth.

In the carrying out of the present method invention, the ore carrying the asbestos fiber to be separated and recovered therefrom is first reduced in any suitable manner to proper size for handling, and as such reduced

ore is fed into what is commonly known as an impact centrifugal mill. Here the reduced ore passes from the center of the centrifugal runner of the mill, and discharging outwardly therefrom, is thrown with considerable force upon or against a circular anvil arranged within the mill, the impact blow thus given to the reduced ore causing a shattering thereof and liberation of the asbestos and a separation of the same from the crushed ore, while the clusters of fiber so released striking against the anvil of the mill is, by the impact blow thereof, shattered and reduced more or less into individual fibers, but without injury to its length and tensile strength. The material thus treated or broken down falls to the bottom portion of the mill and is blown therefrom by the stream of air under pressure and conveyed thereby into a centrifugal separator situated a short distance therefrom and into which the discharge conduit of the mill is extended. In the separator the clusters of fiber not yet reduced to individual fibers are broken up and separated. By introducing the broken up ore material with the separated fiber into the centrifugal separator by an air blast under sufficient conveying pressure, the same is caused to travel around the inside of the annular body of the separator and during such course of travel the remaining clusters of fiber in the mixture become further separated or reduced to individual fibers, the heavier rock or refuse material and sand being thrown centrifugally outwardly and falling by gravity to the bottom of the separator for discharge therefrom, while the lighter fiber is drawn toward the inside of the rotating mass and withdrawn by suction from within the separator through an outlet or exhaust stack leading therefrom. This pneumatic withdrawal of the separated fiber is accomplished by means of an exhaust fan which forces the material into a settling chamber and therefrom into and through a classifier designed to receive the said separated fiber. The dust laden air makes its escape or discharge from the settling chamber through a suitably controlled outlet stack, while the heavier particles or separated fiber is forced by the air under pressure from within the settling chamber into and through the classifier, within which the material settles by specific gravity into

suitable collecting bins arranged to receive the same.

From the foregoing, it will be noted that the fiber or clusters of fiber liberated from the sized ore is treated and conveyed into a centrifugal mill and discharged therefrom and forced through a classifier by air under pressure, and which constitutes the sole medium or transfer vehicle employed for properly disintegrating the mass of mineral fibers into individual fibers and freeing the same of the dirt and foreign material contained therein, whereby the separation and recovery of the mineral fiber is accomplished without injury or damage thereto and without breaking down and destroying the length of the fiber.

The method may therefore be said to reside in the utilization of pneumatic means for primarily breaking up the sized ore to liberate the fiber therefrom, thence transferring the sized ore in its broken down condition to a centrifugal separator for the dividing of the mineral fiber into individual fibers and removing therefrom foreign material adhering thereto, thence transferring the same through the medium of the air pressure to a settling chamber wherein the dust laden air is removed and the separated mineral fiber permitted to settle and be discharged under air pressure into a classifier and within which classifier the separated mineral fibers settle by gravity.

Any suitable form of mechanism may be employed for the mechanical handling of the material, there being illustrated in the accompanying drawings a longitudinal sectional view in side elevation of a suitable apparatus for the carrying out of the desired work, and to which drawing reference should be had.

In the drawings, the numeral 1 is used to designate a bin or hopper for receiving the sized ore to be treated, which ore is delivered by a worm feed 2 into and centrally of a centrifugal mill 3, the fed material falling centrally of the runner 4 within said mill and being thrown outwardly against a die-ring or anvil 5 secured within the mill, the impact blow of the material being sufficient to shatter and break up the ore to liberate the mineral fiber therefrom. The air blast from the mill 3 forces the broken up material through the conduit 7 into the centrifugal separator 8, and into which air is admitted from the outside through the adjustable air inlets 9. The material as delivered within the centrifugal separator is thrown against the inner wall of the separator body 10, which serves to break up the clusters of fiber and reduce the same to individual fibers, the base or refuse material flowing downwardly by gravity and discharging from within the separator through the discharge outlet 11. The air pressure

within the centrifugal separator, draws the liberated mineral fiber towards the center of the separator, from which it is discharged through the uptake 12 and therefrom through the downwardly extended conduit leg 13 into a settling chamber 14, the material being withdrawn from the separator and upwardly through the uptake 12 and downwardly through the conduit extension 13 by means of the exhaust fan 15, which forces the material under pressure into the said chamber 14. The lighter particles and dust flowing with the body of separated fiber discharges from the settling chamber through the outlet stack 16, which is controlled by the regulating damper 17, while the heavier material or separated fiber settles downwardly by gravity and is discharged by the pressure of the flowing air through the outlet conduit 18 into the classifier 19, being carried therethrough by the flowing body of air under pressure, and as moved through the classifier the separated fiber by gravity settles within the series of receiving bins 20 forming the bottom of the classifier, while the dust laden air flowing through the classifier escapes therefrom through the outlet stack 21. The grading of the separated fiber as carried or propelled through the classifier takes place by gravity, although some of the dust carried by the flowing stream of air under pressure passing through the classifier may settle and accumulate in the last of the series of bins.

While I have described a practical and efficient apparatus for the carrying out of the method invention, it will be understood that any suitable form of mechanism may be employed for this purpose just so long as the medium or vehicle for propelling the broken up body of ore throughout the various steps of the process comprises a flowing body of air under pressure, whereby the material under treatment in the various steps of the method is not subjected to a mechanical grinding or crushing action which breaks the fiber and destroys the length thereof.

The described method of milling asbestos ore, cleaning, dusting and classifying the fiber separated from the ore by the utilization of a conveying medium consisting of a flowing body of air under pressure is believed to be new, and it is the desire and wish to claim the same as broadly as the state of the art will warrant.

By the use of the described invention, it will be observed that part of the disintegrated mass of shattered material carrying sand, dust, loose fiber and fiber clusters discharged under air pressure from any suitable type of mill for the shattering thereof, is discharged and introduced into a centrifugal separator by means of an air blast created in any desired manner of sufficient

volume to carry all the material to be delivered to the separator. The rotary motion of the material in the separator further disintegrates the fiber clusters, as well as to force the rock and sand to the outside, the fiber going to the inside of the rotating mass. The suction applied to the separator by means of the exhauster, coupled with a proper introduction of considerably more air into the separator, will draw off the fiber into the discharge pipe of the separator from whence it passes into the exhauster.

The fiber passing to the exhauster will contain some light sand, dust, loose fiber and partly disintegrated fiber clusters. The action in the discharge pipe of the separator and the exhauster is to separate out the light sand and dust, disintegrate what loose fibers remain, and separate from the fiber particles dust still adhering to the same.

Having thus described my invention, what

I claim as new and desire to secure by Letters Patent of the United States is:—

The method of treating fiber bearing ores reduced to a proper size for the separation and recovery of the fiber therefrom, which resides in shattering the ore by an impact blow of the ore to release the fiber therefrom, subjecting the released fiber to the action of air under pressure to permit the baser refuse material to settle out by gravity, subjecting the separated fiber and lighter particles to air under pressure to remove the dust and light particles therefrom and classifying the fiber according to length by forcing the same in a horizontal direction by air under pressure and permitting the discharged fiber to settle by gravity.

In testimony whereof I have signed my name to this specification.

NORRIS K. DAVIS.